

S. D. PADACK,  
ACOUSTIC DIAPHRAGM.  
APPLICATION FILED FEB. 7, 1918.

1,356,399.

Patented Oct. 19, 1920.

Fig. 1



Fig. 2



INVENTOR  
*Simon David Padack*  
BY  
*E. Scherr* ATTORNEY

# UNITED STATES PATENT OFFICE.

SIMON DAVID PADACK, OF BROOKLYN, NEW YORK, ASSIGNOR TO THE AEOLIAN COMPANY, A CORPORATION OF CONNECTICUT.

## ACOUSTIC DIAPHRAGM.

1,356,399.

Specification of Letters Patent. Patented Oct. 19, 1920.

Application filed February 7, 1918. Serial No. 215,880.

To all whom it may concern:

Be it known that I, SIMON DAVID PADACK, citizen of the United States, residing at 28 Hawthorne street, Brooklyn, State of New York, have invented new and useful Improvements in Acoustic Diaphragms, of which the following is a specification.

This invention pertains to acoustic diaphragms particularly for use in phonographs; and in sound-recording and reproducing instruments generally.

In the accompanying drawing is illustrated an acoustic diaphragm which is one of the embodiments that my broad invention is adapted to take. In said drawing, Figure 1 is a face view of the diaphragm; and Fig. 2 is a diagrammatical, enlarged vertical section on the line 2—2 in Fig. 1, the middle portion being shown broken away.

The preferred diaphragm comprises a suitable base such as blotting-paper having incorporated therewith shellac, resin, wax and finely divided glass.

To make it, I prefer to proceed as follows:—I melt together by the use of heat 40% by weight of shellac and 50% of resin. To this I add 10% of powdered glass and thoroughly stir the ingredients. Then I add enough wax to make a considerable layer of it over the surface of the molten mixture, this waxy layer being renewed from time to time, if necessary, as it becomes used up during the next step of the process. This consists in slowly passing blotting-paper through the molten mixture preferably in a long strip, wider than the finished diaphragms. The forward end of the strip as it emerges from the bath then passes between heated pressure-rolls, which complete the impregnation of the blotting-paper with the shellac and resin and force the powdered glass into the paper. At the same time the rolls remove the excess material and compress the paper, making it denser and harder. As the strip passes through the waxy layer from the molten mixture to the rolls, it carries with it a considerable quantity of the wax which becomes incorporated with the paper strip as it passes through the rolls, especially at the surface of the paper, the wax being preferably the last ingredient to be applied.

After a short interval the individual dia-

phragms can be cut from the strip by the use of cutting dies or the like. The resulting diaphragms used in phonograph sound-boxes give excellent reproductions.

Changes can be made in the above process, the ingredients and their proportions which will still be within the spirit of the invention and by such suitable modifications diaphragms can be made which will nevertheless be within my invention and the annexed claims.

The shellac and resin constitute broadly a binder besides making their own several contributions to the properties of the preferred diaphragm. The glass contributes to the brilliancy and other desirable acoustic properties of the diaphragm. While glass is preferred, it is possible to employ other finely divided vitreous material such as silica, obsidian, etc., or in general any mineral which is insoluble in the binder and has sonorous qualities similar to glass. The diaphragm is not materially affected by dampness and to this quality the wax contributes. Instead of blotting-paper, any other suitable base may be used, but preferably it should be porous or absorbent. Depending on the precise acoustic quality desired for the diaphragms, the above process can be made longer or shorter in duration so as to impregnate the base more or less completely from its surface layers inwardly to its center layer or zone.

However, the diaphragm I prefer is the one which is not impregnated to the center zone. In this preferred diaphragm the resin and shellac penetrate from each surface of the disk about  $\frac{1}{4}$  or so through the thickness of the disk, and the powdered glass ingredient penetrates from the surface about  $\frac{1}{3}$  the penetration of the resin and shellac. This embodiment of my invention is illustrated diagrammatically in the drawing wherein in Fig. 2, A for example, designates the entire thickness of the paper base, B the surface layers impregnated with the resin and shellac, C the shallower surface layers containing embedded therein the powdered glass material in addition to the resin and shellac, and finally D designates the unimpregnated central zone of the base.

What I claim is:

1. An acoustic diaphragm comprising a

55

60

70

75

80

85

90

95

100

105

- suitable base having powdered glass combined therewith.
2. An acoustic diaphragm comprising a suitable base having finely divided vitreous material combined therewith.
3. An acoustic diaphragm comprising powdered glass and a binder incorporated with a suitable base which is absorbent to the binder.
- 10 4. An acoustic diaphragm comprising a resonant moisture proof binder, a suitable absorbent base therefor, and powdered glass, the binder and glass being absorbed and pressed into the surface of the base.
- 15 5. An acoustic diaphragm comprising a suitable base having shellac, powdered glass, and resin incorporated therewith.
6. An acoustic diaphragm comprising a suitable base having shellac, a finely divided mineral and resin incorporated therewith, the mineral having sonorous qualities similar to glass.
- 20 7. An acoustic diaphragm comprising a suitable base having shellac, powdered glass, wax and resin incorporated therewith.
8. An acoustic diaphragm comprising a suitable base having shellac, a finely divided mineral, wax and resin incorporated therewith, the mineral having sonorous qualities similar to glass.
- 25 9. An acoustic diaphragm comprising a suitable base having vitreous material, shellac and resin incorporated therewith.
10. An acoustic diaphragm comprising a suitable base having finely divided vitreous material, shellac, wax and resin incorporated therewith.
11. An acoustic diaphragm comprising a suitable base having incorporated therewith a binder of resonant material, a wax and a finely divided mineral insoluble in the binder.
12. An acoustic diaphragm comprising a suitable base having incorporated therewith shellac, resin and a finely divided mineral insoluble in the shellac and resin and having sonorous properties similar to glass.
13. An acoustic diaphragm comprising a suitable base whose surface layers only are filled with a finely divided vitreous material and whose surface layers are also impregnated with a binder which extends through and below the vitreous material, leaving the central zone of the base unimpregnated.
14. An acoustic diaphragm comprising a suitable base of fibrous material having finely divided, hard, sharp vitreous material embedded in its surface.
- In testimony whereof I, said SIMON DAVID PADDACK have signed my name to this specification this 5th day of February, 1918.
- SIMON DAVID PADDACK.